

## UNITED STATES PATENT OFFICE

2,291,718

## VISCOSE SPINNING PROCESS

Emil Hubert, Dessau-Ziebigk, Adolf Hamann,  
Wolfen Kreis Bitterfeld, and Karl Weisbrod,  
Dessau, Germany, assignors, by mesne assignments,  
to Walther H. Duisberg, New York,  
N. Y.

No Drawing. Application June 6, 1939, Serial No.  
277,626. In Germany June 7, 1938

3 Claims. (Cl. 18—54)

This invention relates to a spinning process for viscose rayon.

It is known that artificial threads of very good physical constants, especially high tenacity, can be produced by stretching viscose threads in a highly swollen and highly plastic condition. For making such threads there are used spinning baths of high acid concentration, preferably sulphuric acid baths (U. S. Patent No. 1,683,199) or solutions of strong acids and salts (British Patent No. 345,938). It has also been proposed to divide the spinning operation into two stages, namely a coagulation by means of agents having only a coagulating effect and a plasticisation of the coagulated thread with subsequent final decomposition to cellulose hydrate; the threads are stretched in a plastic condition (British Patent No. 298,548).

These known processes have the disadvantage that they require strongly acid baths for attaining good results, so that in practice they give rise to difficulties of various kinds. Besides the use of these strong acid baths it has been proposed to attain similar effects by using sulphuric acid solutions of especially low percentage strength, for example 0.5—7 per cent of sulphuric acid (British Patent No. 309,053). However, these baths have the disadvantage that the plastic condition of the thread persists for only a few seconds so that it is difficult to be sure of taking advantage of this transitory condition for the stretching.

The present invention is based on the observation that a plasticizing agent may be added to the coagulation bath with the result that the threads obtained can be well stretched and are then of good tenacity.

The invention consists in a process in which the threads are coagulated in a bath free of acid and containing a non-acid plasticizing agent, for instance urea, thiourea, ammonium thiocyanate or the like, the coagulated thread being stretched and finally decomposed to cellulose hydrate. Preferably the coagulation bath should be one containing not more than 50 per cent of water.

The decomposition to cellulose hydrate may occur under stretching or wholly without stretching, for example after the thread has been cut into staple fiber. As decomposing baths there may be used solutions of acids alone or of acids and salts, for instance the known Müller bath. The decomposition may also be a thermal effect, for example the thread may be subjected to a hot liquid or hot vapor which is especially useful in case of cut staple fiber.

The following examples illustrate the invention:

*Example 1.*—From a normally ripened viscose having for example 7.5 per cent of cellulose and 6.5 per cent of alkali there is spun a thread having a single titer of 2.6 denier from a spinneret having 120 perforations each of 0.08 millimeter diameter into a bath containing 8.5 per cent of  $\text{Na}_2\text{SO}_4$ , 16 per cent of  $(\text{NH}_4)_2\text{SO}_4$  and 39 per cent of urea the bath having a temperature of 60° C. The threads issuing from this bath are drawn over glass rods arranged to afford a zig-zag path, the draught being 40 meters per minute.

The coagulated and stretched threads are cut to staple length and decomposed in boiling sodium sulphate solution. The staple fibers are desulfurized in the usual manner and then soaped. The fibers thus spun have a good extension and a very good tenacity:

20 Dry tenacity: 3.8 per denier, extension 19 per cent.

Wet tenacity: 2.74 per denier.

The coagulation bath may have a composition different from that described in this example. Preferably however the bath should not contain more than 50 per cent of water. Baths of the following composition also give good results:

25 5.5 per cent of  $\text{Na}_2\text{SO}_4$ , 19 per cent  $(\text{NH}_4)_2\text{SO}_4$ , 34 per cent urea, or 15 per cent of  $\text{Na}_2\text{SO}_4$ , 9 per cent  $(\text{NH}_4)_2\text{SO}_4$ , 35 per cent of urea.

*Example 2.*—A thread of single titer 2 (spinneret having 120 perforations each of 0.08 millimeter diameter) is spun from a normally ripened cellulose containing 7.5 per cent of cellulose and 6.5 per cent of alkali in a bath containing 10 per cent of  $\text{Na}_2\text{SO}_4$ , 13 per cent of  $(\text{NH}_4)_2\text{SO}_4$  and 33 per cent of urea maintained at 50° C. The thread is stretched over several glass rods set to form a zig-zag path and is wound at the rate of 50 meters per minute on a spool. For decomposing the threads to cellulose hydrate the spool runs during the spinning in an acid upper bath containing 13 per cent of sulfuric acid and 28 per cent of sodium sulfate. The acid spool is further treated in the usual manner, for example de-acidified in a suction washer and desulfurized in the form of hanks and then bleached and soaped.

40 45 Dry tenacity: 3.3 per denier, extension 6 per cent. Wet tenacity: 2.1 per denier, extension 5.5 per cent.

We claim:

50 55 1. A process of producing viscose threads which

comprises spinning viscose into an aqueous acid-free bath incapable of entirely decomposing the cellulose xanthate, but capable of coagulating the viscose, said bath containing about 10 per cent sodium sulfate and about 13 per cent ammonium sulfate and about 33 per cent of urea, stretching said threads while in plastic condition and decomposing the cellulose xanthate to cellulose hydrate.

2. A process of producing viscose threads which comprises spinning viscose into an aqueous acid free bath incapable of entirely decomposing the cellulose xanthate, but capable of coagulating the viscose, said bath containing sodium sulfate, ammonium sulfate and urea in such quantities as to amount to more than 50% of the bath, stretch-

ing the threads while in plastic condition and decomposing the cellulose xanthate to cellulose hydrate.

3. A process of producing viscose threads which comprises spinning viscose into an aqueous bath free from acids, incapable of decomposing the cellulose xanthate but capable of coagulating the viscose, said bath containing sodium sulfate, ammonium sulfate and urea in such quantities as to amount to more than 50% of the bath, stretching the threads after leaving the bath, cutting off the threads in staples and decomposing the staple waste in hot solution or hot vapors.

EMIL HUBERT.  
ADOLF HAMANN.  
KARL WEISBROD.